

Patented Oct. 10, 1922.

1,431,225

# UNITED STATES PATENT OFFICE.

CHARLES JASON GREENSTREET, OF CHICAGO, ILLINOIS.

## FUEL PRODUCT AND METHOD OF MAKING SAME.

No Drawing.

Application filed May 9, 1922. Serial No. 559,600.

To all whom it may concern:

Be it known that I, CHARLES JASON GREENSTREET, a citizen of the United States, residing at Chicago, in the county of Cook and State of Illinois, have invented certain new and useful Improvements in Fuel Products and Methods of Making Same, of which I declare the following to be a full, clear, and exact description.

10 This invention relates to a fuel product and a method of making the same and, more particularly, to a fluid fuel composed of a liquid fuel and finally divided solid fuel particles suspended therein in a substantially permanent suspension.

15

The many advantages in the use of fluid fuels such as their low labor cost in firing, their freedom from ash, the exact control of the rate at which they may be supplied and 20 burned and the exact proportioning of air to fuel which is possible with them and the high efficiency and economy which these features make possible, have made the prospect of transforming solid fuels into liquid 25 fuels highly attractive and desirable. This is more particularly the case as a large amount of solid fuel is produced in the form of dust, powdered and small dimensioned particles, such as culm, which are difficult 30 to burn on the ordinary types of grates and therefore have little commercial value. Certain fuels, such as lignite, which disintegrates to a powder on exposure to the atmosphere, can not be readily handled and 35 burned in the solid form are of little use and value.

Attempts have been made to utilize powdered fuels of the above types by simply mixing them with fluid or liquid fuels to serve as 40 a vehicle or carrier and burning the mixture similarly to a liquid fuel. The densities of these fuels are, however, generally different from those of the liquid fuels which are available, and the solid particles settle out 45 after standing for a short time and form hard cakes which clog the conduits and passages of fluid fuel burning apparatus. Attempts to reduce the coal particles to a 50 size approaching colloidal dimensions, while offering possibilities in the way of stability of suspension, are not commercially feasible or practicable since the excessively fine grinding which this requires makes the cost 55 of the fuel prohibitive.

An object of the present invention is to

provide a fuel product in which solid fuel particles of a size readily and cheaply obtainable by ordinary grinding are suspended in a substantially stable, uniform 60 suspension in a fluid fuel medium.

Another object of the invention is to provide a fluid fuel product comprising solid particles above colloidal dimensions suspended in a liquid fuel medium treated to 65 render it resistant to the settling or separation of said particles.

A further object of the invention is to provide a method of forming a substantially permanent suspension of solid fuel 70 particles of above colloidal size in a fluid fuel medium.

Further objects of the invention are to provide a fuel product in which solid fuel particles are maintained in suspension in a 75 fluid fuel medium by the emulsification of a suitable fuel oil and water and a method of maintaining a suspension of such particles in a fluid fuel medium by the emulsification of fuel oil and water and of a 80 method of stabilizing such emulsions by the use of soaps.

With these and other objects in view, the invention comprises the fuel product and 85 the method of making the same described and set forth in the following specification and claims.

In the present invention the solid fuel is reduced by any suitable grinding means 90 available for grinding on a commercial scale, to a sufficient degree of fineness so that the particles may readily pass through the passages of the fuel burning apparatus without danger of clogging. The fuel is 95 preferably ground as fine as is practicable with ordinary commercial methods, since the finer the grinding the more easily may the particles be maintained in suspension, but grinding to a degree approaching colloidal dimensions is not necessary. The finely divided solid fuel particles are then 100 uniformly dispersed and suspended in a liquid fuel medium in the quantity desired for the particular purpose in view. To fix 105 or stabilize this suspension the liquid fuel medium is rendered sufficiently dense and viscous to resist or overcome the tendency of the solid particles to settle out of the liquid under the action of gravity. This 110 stabilization is preferably obtained by incorporating into the liquid fuel a substance

which increases its density and viscosity such, for example as a liquid or semi-liquid which forms a permanent or substantially permanent emulsion with the oil. A suitable emulsifying agent or protective agent 5 may also be added, when necessary to stabilize and maintain the emulsion.

The solid fuel used in forming the fuel product may be any kind which can be reduced to a degree of fineness that it will 10 pass through the burner apparatus in which the fuel is to be burned. Anthracite and bituminous coals, coal dust, coke, coke dust, lignite, saw dust and other carbonaceous 15 and cellulosic waste products may be mentioned as sources of the solid fuel. If not already in the form of a sufficiently fine powder these materials are pulverized in any of the usual mills or grinding devices used 20 for the production of powered fuels which will provide a powder of the desired degree of fineness. Any mill which grinds to a fineness of about two hundred mesh or finer is usually satisfactory for this purpose. The 25 finer the grinding the more desirable the resulting fuel from many standpoints, but the excessively fine grinding necessary to reduce the solid fuel to colloidal dimensions is not required. Two or more kinds of fuel 30 may be used to produce a fuel having certain desired properties or to utilize waste products which do not give desirable results when used alone or which are not available in sufficient quantities to provide the required quantity of fuel.

Any liquid fuel which may be thickened or increased sufficiently in density or viscosity may be used as the liquid fuel medium. The mineral fuel oils which are obtained as 40 the heavy residues in the refining of petroleum or in the cracking of hydrocarbon oils in pressure stills or other cracking processes are especially suited for the present fuel product as they are available in large quantities, 45 have a considerable initial gravity and viscosity and are readily emulsifiable. The heavier grades of Mexican crude petroleums and the residues from the refining of such oils and from cracking of their lighter 50 distillates are also very desirable for the present purpose. Fuel oils of a density of about 25° Bé. or denser have been found very satisfactory as a liquid fuel medium. Certain of the naturally occurring emulsions or 55 "bottom settling" which are not suitable for refining on account of their water content may be utilized in the present fuel.

Water has been found to be a suitable emulsifying component for oils of this type. 60 The water may be in the condition of purity in which it occurs or may have added to it certain materials to render its emulsion with the fuel oil more stable. The ground water or surface waters which are produced with 65 certain crude petroleums are usually suitable.

Other materials may be used in forming the emulsion but when possible water is preferred as the main constituent of the emulsifying constituent because of its cheapness and its property of promoting a smokeless combustion of the fuel. 70

When, under certain conditions, there is a tendency for the emulsion to become unstable and to separate into its constituents, a small amount of a stabilizing agent may 75 be added. For this purpose a soap solution is generally suitable. As an example a solution of from ten to fifty per cent of ordinary soap or tar soap dissolved may be used as the emulsion stabilizer. Or a suitable soap 80 may be made by boiling five parts of animal fat, such as packing house wastes and similar cheap products, with ten parts of a caustic solution. The soap solution may be used in full strength as the emulsifying constituent 85 or may be added to or diluted with water as conditions may require or the cost of materials may render desirable.

The fuel is preferably formed by mixing the finely powdered fuel with the fluid fuel 90 medium in a mixing device or in a tank arranged to permit of air agitation or fitted with suitable stirring devices. The emulsifying constituent is then agitated with the solid and liquid fuel mixture to produce the 95 emulsion, a stabilizing agent such as the soap solution being used or added to the water to assist in forming the emulsion when required. Some or a considerable part of the emulsifying constituent may be present when 100 the solid fuel is being suspended in the liquid fuel medium, particularly when a natural emulsion or bottom settling is being used. The emulsion may be obtained in a thick liquid or paste or may be thickened until 105 it is in the form of a solid or semi-solid paste or gel which may be sufficiently liquefied when warmed slightly, to be pumped to and through the burner apparatus. When a very heavy fuel oil is used the resulting 110 emulsion with water or a heavy solution the density is increased to materially lessen the action of gravity on the solid fuel particles and assist in maintaining the particles in suspension. 115

As an example of a specific form of embodiment of the invention thirty-three parts of suitably powdered coal is suspended in one hundred parts of fuel oil of 22° Bé. gravity by air agitation in a tank. Two parts of 120 soap dissolved in just sufficient water to make a jelly is then added and the whole further agitated until homogeneous. A fuel oil of 18° Bé. was also found to work satisfactorily when emulsified. 125

The fuel product obtained as above may be used in substantially the same manner as the ordinary types of heavy fuel oils and for substantially the same purposes. In addition to utilizing many fuels which are at 130

present wasted it permits of a fuel of any desired quality to be obtained and requires less storage space and is more free from fire dangers than the ordinary types of fuels.

5 This application is a continuation in part of my co-pending applications Serial No. 274,358 filed January 31, 1919 and Serial No. 312,871 filed July 23, 1919 to the extent of some of the subject matter disclosed in said 10 applications and also disclosed herein.

Having described the invention, what I claim and desire to secure by Letters Patent is:

15 1. A fluid fuel product which comprises a liquid fuel and a powdered fuel dispersed throughout said liquid fuel and of a size at which it settles out of said liquid fuel, and said liquid fuel being thickened through emulsification to avoid settling of said powdered fuel.

20 2. A process of making a fuel product which comprises mixing powdered fuel with a fluid fuel said fuel powder being of a size at which it settles from said fluid fuel, and thickening said fluid fuel to avoid the settling of said powdered fuel.

25 3. A fuel product which comprises a liquid fuel, solid fuel particles dispersed throughout said liquid fuel and of a size at which they settle out of said liquid fuel, and a material of greater density than said liquid fuel emulsified in said liquid fuel to produce a stiff, heavy medium and to avoid settling of said solid particles.

35 4. A fuel product which comprises a liquid fuel, a powdered fuel dispersed throughout said liquid fuel and of a size at which it settles out of said liquid fuel, and water emulsified in said liquid fuel, said liquid fuel being thickened through said emulsification to avoid settling of said powdered fuel.

50 5. A fuel product which comprises a liquid fuel, a powdered fuel dispersed throughout said liquid fuel and of a size at which it settles out of said liquid fuel, water emulsified in said liquid fuel to thicken said fuel and avoid the settling of said powdered fuel and a material to stabilize said emulsion of water and liquid fuel.

55 6. A fuel product which comprises a liquid fuel, a powdered fuel dispersed throughout said liquid fuel and of a size at which it settles out of said liquid fuel, and a soap solution emulsified in said liquid fuel to thicken said liquid fuel and avoid the settling of said powdered fuel.

60 7. A fuel product which comprises a fuel oil of a density of 25° Be' or lower, a powdered fuel dispersed throughout said fuel dispersed throughout said fuel oil and of a size at which it settles out of said fuel oil, and water emulsified in said oil to thicken said oil and avoid the settling of said powdered fuel.

8. A fuel product which comprises a fuel oil of a density of 22° Be', a powdered fuel dispersed throughout said fuel oil and of a size at which it settles out of said fuel oil, and water emulsified in said oil to thicken 70 said oil and avoid the settling of said powdered fuel.

9. A fuel product which comprises approximately 100 parts of fuel oil, approximately 33 parts of powdered fuel dispersed 75 through said fuel oil and of a size at which it settles out of said fuel oil, and approximately 10 parts of water emulsified in said oil, said fuel oil being thickened through said emulsification to avoid settling of said 80 powdered fuel.

10. A fuel product which comprises approximately 100 parts of fuel oil, approximately 33 parts of powdered fuel dispersed through said fuel oil and of a size at which 85 it settles out of said fuel oil, and approximately 10 parts of soap solution emulsified in said oil, said fuel oil being thickened by said emulsification to avoid settling of said powdered fuel.

90 11. A fuel product which comprises approximately 100 parts of fuel oil, of a gravity of approximately 22° Be', approximately 33 parts of powdered fuel dispersed throughout said oil and of a size at which it settles 95 out of said fuel oil and approximately 10 parts of water emulsified in said oil, said oil being thickened by said emulsification to avoid settling of said powdered fuel.

12. A process of making a fuel product 100 which comprises mixing powdered fuel with a liquid fuel, said powdered fuel being of a size at which it settles out of said liquid fuel, and thickening said liquid fuel by emulsifying with a thickening agent to 105 maintain said powdered fuel suspended in said liquid fuel.

13. A method of forming a fuel product which comprises suspending a powdered solid fuel in a liquid fuel by gaseous agitation, said powdered fuel being of a size 110 at which it settles from said liquid fuel, and thickening said liquid fuel by emulsification with water.

14. A method of forming a fuel product 115 which comprises suspending a powdered fuel in a liquid fuel by gaseous agitation, said powdered fuel being of a size at which it settles from said liquid fuel, and thickening said liquid fuel with water and soap 120 as an emulsion stabilizer.

15. A method of forming a fuel product which comprises mixing and suspending a powdered fuel, said powdered fuel being of a size at which it settles from said liquid 125 fuel, in a fuel oil of 25° Be. gravity or less and thickening by emulsifying said fuel oil with water.

16. A process of making a fluid fuel product which comprises forming a mixture in 130

cluding a heavy liquid, a lighter liquid fuel relatively immiscible in said liquid and suspending a finely divided solid fuel in said liquid mixture, the particles of said solid fuel being of a size at which they settle from said liquid fuel and the consistency of the resulting liquid mixture being such as to prevent substantial settling and separation of said particles from said liquid.

10 17. A fuel product which comprises a

fluid fuel, a liquid to render the consistency of the mixture such as to receive and hold a solid fuel in substantially permanent suspension and a powdered fuel of a size which will not readily mix and remain suspended in said fluid fuel, said powdered fuel dispersed throughout said fluid fuel.

In testimony whereof, I affix my signature.

CHARLES JASON GREENSTREET.